

Oct. 20, 1931.

W. MENDEL

1,828,374

METHOD OF TRADE MARKING CARBON PAPER

Original Filed June 6, 1929

FIG. I.



FIG. II.



INVENTOR:

WILLIAM MENDEL,  
By Arthur E. Peigley  
Attorney.

## UNITED STATES PATENT OFFICE

WILLIAM MENDEL, OF BEVERLY, NEW JERSEY

## METHOD OF TRADE MARKING CARBON PAPER

Original application filed June 6, 1929, Serial No. 368,993. Divided and this application filed June 30, 1930. Serial No. 404,956.

This is a division of my application Serial No. 368,993 filed June 6, 1929, for Letters Patent of the United States No. 1,769,592 granted July 1, 1930, for method of trade-marking carbon paper, wherein the method herein disclosed is generically claimed.

My invention relates to the manufacture of transfer webs of tissue paper and the like coated with transfer material, which is known to the trade as "dope", and preferably a mixture of waxes, oils, and pigment, such as lamp black, if the material is to be used for what are called "carbon copies" from written impressions.

Commercial competition with respect to such products is such that it is highly desirable to mark each sheet in such a manner as to clearly manifest thereon the origin thereof, to prevent substitution of cheaper products by unscrupulous dealers. It is also desirable to distinguish such products as to quality thereof and as to the capacity of the respective sheets for production of transfer impressions. For instance, distinct marks upon such products may respectively indicate the manufacturer thereof and the grade of the product, and the maximum capacity of the respective sheet as to the number of copies which may be simultaneously made with such sheets.

It has long been the practice to identify paper products with what are termed "water marks", i. e., regions of the paper which are reduced in thickness while the paper is wet. However, such marking is not only costly but, in the extremely thin tissues used for transfer purposes, such marking lessens the value of the product by causing perforations in the tissue. Printers' ink imprints upon such tissues also render them liable to break at the edges of the imprints and renders them less capable of transferring impressions throughout the area covered by such imprints. It has also been proposed to apply to the faces of the tissues from which transfer webs are to be formed, a penetrating marking fluid which penetrates from the coated side of the paper to the uncoated side so as to be visible from the back of the paper and is of such nature as to resist absorption of the transfer coat-

ing throughout the area of the tissue thus penetrated. The effect of such a method and means of trade-marking a transfer web is that, as seen from the back, the area marked is of a lighter tint or shade than the surrounding area, which has absorbed the oils and waxes from the carbon dope.

It is the purpose and effect of my invention to mark such transfer webs with a chemical which imparts to the material of the web a greater capacity for absorption of the oily substances from the dope coating than the areas of the web which are not thus treated, and with the effect that, as seen from the back, the marked area is darker in tint or shade than the surrounding area.

My invention includes the various novel features of method and means hereinafter more definitely specified.

In said drawings; Fig. I is a perspective view of the back of a sheet of transfer web trade-marked in accordance with my invention.

Fig. II is a fragmentary elevation of a portion of the back of a transfer web trade-marked in accordance with my invention and having additional marks respectively designating the quality and the capacity of the same.

In Fig. I, I have shown a sheet of carbon paper 1 manifesting the trade-mark 2 by outlines 3 which are darker than the surrounding area 4 of the back of the sheet of tissue, provided with a dope coating upon its opposite face. Such marking is preferably effected by applying, throughout the lines 3, a cellulose nitrate solvent, preferably having a high boiling point and low volatility; and particularly derivatives of ethylene glycol and diethylene glycol; for instance, ethylene glycol mono ethyl ether acetate, diethylene glycol mono butyl ether, etc. Such chemicals have the capacity to render the tissue paper of the sheet 1 more absorbent of the oily part of the dope, where treated therewith than where it is not thus chemically treated.

In Fig. II, the transfer web 6 is provided with marks 7, 8, and 9, by the initial application to the web of a chemical capable of increasing the absorbing capacity of the web

as aforesaid. However, said marks are for respectively different purposes; the mark 7 indicating the manufacturer; the mark 8 indicating the grade of the product; and the 5 mark 9 indicating the capacity of the product as to the number of transfer copies which may be simultaneously made therewith from a single typewritten imprint. As indicated, each of said marks 7, 8, and 9 is darker than 10 the surrounding area 10 of the web 6.

The contrast between the chemically treated area and the other areas of the transfer webs may be varied in accordance with the treatment of the latter after the transfer 15 coating is applied thereto. For instance, the coated web may be passed over heated cylindrical rolls to cause the waxy, oily portion of the dope to be absorbed, more or less, by the web tissue, according to the use to be made of 20 the transfer web. The coating is applied hot, and if instantly chilled upon the surface of the web, absorption of the latter is minimized and impressions transferred therefrom are as dark as possible and, in fact, such 25 chilled coating may come off with a single impression, whereas, in accordance with the degree of absorption, the impressions are fainter, and more of them can be made.

The degree of absorption is variable in accordance with several factors, for instance, 30 the temperature of the hot roll over which the web passes, the speed of its passage, and the area of contact of the web and the roll during such passage.

35 It is important to note that, under such conditions of manufacture, applying to the tissue to be used for forming a transfer web, any material for trade-marking purposes, or otherwise, which resists absorption of the 40 waxy, oily substances from the dope, interferes with the grading of the product by the heat treatment aforesaid in that such treatment is ineffective in causing such absorption throughout the areas thus marked. On the 45 contrary, the use of my invention leaves all of the tissue with at least its initial capacity for absorption as aforesaid.

Although I have specified lamp black as a 50 pigment and that is the principal ingredient of the transfer dope in what is known to the trade as carbon paper, there is a commercial demand for colored transfer material, and it is to be understood that my invention may be advantageously employed in the manufacture 55 of transfer webs of any color. For instance, the dope may include more or less of a pigment known to the trade as "Victoria blue base" in accordance with the tint or shade of blue desired. In manufacturing such colored products, the trade-marking may be effected with similar or contrasting colors. For 60 instance, if the webs are to be coated with dope colored with Victoria blue base, some of the latter may be mixed with the cellulose nitrate solvent before the latter is applied.

For instance, I have found it convenient to use a mixture of 95% ethylene glycol mono ethyl ether acetate with 5% Victoria blue base, which colors the web, before the colored dope is applied thereto.

As a matter of economy and control of the solvents aforesaid, they may be mixed with diluents. For instance, ethylene glycol mono ethyl ether acetate and similar derivatives of ethylene glycol may be diluted with water. 70 However, I prefer to employ a more volatile diluent, such as carbon tetrachloride or other liquid hydrocarbons. Although gasoline and naptha may be used in lieu of carbon tetrachloride as diluents of cellulose nitrate solvents; carbon tetrachloride is preferable because it is not inflammable like the other hydrocarbons aforesaid.

80 For example, twenty per cent., of ethylene glycol mono ethyl ether acetate, or other derivative of ethylene glycol, may be diluted with eighty per cent., of carbon tetrachloride, and applied to the surface of the web by any convenient method or means.

85 However, in any case, it is characteristic of the use of my invention that the trademarked portion of the transfer web is darker than the surrounding area, instead of lighter, as in the prior art, exemplified, for instance, by Letters Patent of the United States No. 1,513,246 dated October 28, 1924, and No. 1,659,320 dated February 14, 1928, granted to William Jonse Hughes, describing and claiming processes of marking paper by rendering a portion of the area thereof less than 90 normally absorbent of the oily portion of the transfer material.

95 Therefore, I do not desire to limit myself to the precise details of procedure or means for effecting my invention herein set forth, as it is obvious that various modifications may be made therein without departing from the essential features of my invention, as defined in the appended claims.

100 I claim:

11 1. The process of marking carbon paper, which process consists in applying the desired design to the supporting paper or tissue with a cellulose nitrate solvent including ethylene glycol mono ethyl ether acetate.

11 2. The process of marking a transfer web which consists in applying thereto a neutral chemical including a product of reaction of an acid which is capable of increasing the capacity of the web for absorption of waxy, oily transfer material, and then applying such transfer material to said web.

12 In testimony whereof, I have hereunto signed my name at Burlington, New Jersey, this twenty-eighth day of June, 1930.

12 WILLIAM MENDEL.